

3,198,739

## LUBRICANTS AND POLYMERIC ADDITIVES THEREFOR

Harry F. Richards, Concord, Calif., Stephen A. Herbert, Jr., Weston, Conn., and Robert J. Moore, Orinda, Calif., assignors to Shell Oil Company, New York, N.Y., a corporation of Delaware  
No Drawing. Filed Nov. 25, 1960, Ser. No. 71,403  
4 Claims. (Cl. 252—56)

This invention relates to improved mineral oil lubricating compositions and to an improved oil-soluble polyhydroxy-carboxylate copolymer therefor.

It is known that certain nitrogen-containing polymer compounds such as the commercial additives LOA-564 and 565 of Du Pont or Rohm and Haas 900 Series Acryloids such as Acryloid 917 or 966 as well as others, are good detergent additives for lubricating oil compositions. Such detergent nitrogen-containing polymeric additives lack wear-inhibiting properties and therefore oils which contain them must be supplemented with wear inhibitors or extreme pressure agents, etc. These materials and the acidic materials formed during engine operation tend to interact with the polymeric nitrogen-containing detergents, resulting in sludge and corrosion.

It is an object of the present invention to provide an improved oil-soluble detergent copolymer. Another object of the invention is to provide a lubricating oil composition possessing good detergent and antisludging properties. Still another object of the invention is to provide a lubricating oil composition containing a novel oxygen-containing copolymer which possesses good detergent and anti-sludging properties. Other objects in accordance with the invention will be apparent hereinafter.

It has now been discovered that these and other objects of the present invention may be accomplished by a new and novel copolymer having essentially a long linear hydrocarbon backbone chain and attached thereto, in a random or uniform fashion, two essential groups, the first being an oil-solubilizing ester group —COOR where R is a C<sub>10-20</sub> alkyl radical, preferably a C<sub>12-18</sub> alkyl radical, and the second being a —COOR'—OH group where R' is a C<sub>5-7</sub> alkyl radical. Polymers of this type may be represented by the Formula I



where R and R' are alkyl radicals as defined above, Y may be a C<sub>12-20</sub> alkyl radical or a polar radical such as an ester, amide, amine, or phosphate radical or the like, m and m<sub>1</sub> are whole numbers of at least 2 each and n may be zero or a whole number, the ratio of m to m<sub>1</sub> may vary from 1:10 to 10:1, preferably from 5:1 to 2:1 and the ratio of m+m<sub>1</sub> to n when n is a whole number may vary from 10:1 to 5:1, respectively. The molecular weight of the polymer varies from about one thousand to about one million, preferably from 10,000 to 500,000.

The first polymerizable monomer group includes acrylic and alkacrylic esters of aliphatic alcohols of at least 8 carbon atoms, preferably of from 10 to 20 carbon atoms, and include, inter alia, decyl acrylate, lauryl acrylate, stearyl acrylate, eicosanyl acrylate, docosanyl acrylate, decyl methacrylate, lauryl methacrylate, cetyl methacrylate, stearyl methacrylate, and the like, and mixtures thereof.

The other polymerizable group includes omega-hydroxy-esters of acrylic or alkacrylic acid and dihydroxy alkanes which may be straight or branch-chain, preferably alpha,

omega-dihydroxy alkane such as alpha-omega-ethylene glycol (1,5-pentanediol), alpha,omega-hexylene glycol, alpha,omega-heptylene glycol, neopentyl glycol, etc. Such esters include omega-hydroxyamyl acrylate, omega-hydroxyamyl methacrylate, omega-hydroxyhexyl acrylate, omega-hydroxyhexyl methacrylate, omega-hydroxyheptyl acrylate, omega-hydroxyheptyl methacrylate, 1,3-di-methyl-3-hydroxybutyl methacrylate and mixtures thereof.

- 5 10 The polymerizable monomer (Y) which is an optional component in copolymers of the present invention may include polyene hydrocarbons such as alpha-unsaturated long-chain hydrocarbons, unsaturated esters, unsaturated amides, e.g., such as dodecene-1, tridecene-1, tetradecene-1, hexadecene-1, heptadecene-1, octadecene-1, tritriacontene-1, tetratriacontene-1, heptacontene-1, 4,4-dimethyl-1-decene-1, 5,5,7,7-tetramethyl-decene-1, etc., vinyl esters e.g., vinyl laurate, vinyl tridecanoate, vinyl myristate, vinyl pentadecanoate, vinyl 15 palmitate, vinyl margarate, vinyl stearate, vinyl nonadecanoate, vinyl arachidate, vinyl behenate, vinyl 4,5,6-trimethyl-dodecanoate, vinyl 6,8,9-triethyltridecanoate, vinyl 12-hydroxystearate, vinyl 9,10-dihydroxystearate, vinyl chlorostearate, vinyl cyanostearate, vinyl acetylstearate; 20 vinyl ethers, vinyl dodecyl ether, vinyl tridecyl ether, vinyl tetracosyl ether, vinyl hexacosyl ether; allyl esters or ethers, allyl stearate, allyl dodecyl ether; amido esters, e.g., N-lauryl methacrylamide, N-stearyl methacrylamide, N,N-distearyl methacrylamide; vinylpyridines, e.g., 4-25 vinylpyridine, 2-methyl-5-vinylpyridine, vinylpyrrolidone, vinyl phosphonates and allyl phosphates, e.g., trimethylallyl phosphate, bis-chloroethyl vinyl phosphonate and mixtures thereof.

The polymerization may be effected in the presence of a substantially inert liquid and in the presence of an oxygen-yielding catalyst at a temperature in the range of 50 to 150° C., preferably between 60-90° C.

- 35 Suitable liquid reaction media are various classes of hydrocarbons or their mixtures which are liquid and substantially inert under the polymerization conditions of the present process. Certain classes of aliphatic hydrocarbons can be employed as a liquid hydrocarbon reaction medium in the present process. Thus may be employed various saturated hydrocarbons (alkanes and cycloalkanes) which are liquid under the polymerization reaction conditions and which do not crack substantially under the reaction conditions. Either pure alkanes or cycloalkanes or commercially available mixtures, freed of catalyst poisons, may be employed. For example, 40 we may employ straight run naphthas or kerosenes containing alkanes and cycloalkanes. Specifically, we may employ liquid or liquefied alkanes such as n-pentane, n-hexane, 2,3-dimethylbutane, n-octane, iso-octane (2,2,4-trimethylpentane), n-decane, n-dodecane, cyclohexane, 45 methylcyclohexane, dimethylcyclopentane, ethylcyclohexane, decalin, methyldecalins, dimethyldecalins and the like.

Members of the aromatic hydrocarbon series, particularly the mononuclear aromatic hydrocarbons, viz., 50 benzene, toluene, xylenes, mesitylene and xylene-p-cymene mixtures can also be employed. In addition, we may employ such aromatic hydrocarbons as ethylbenzene, isopropylbenzene, sec-butylbenzene, t-butylbenzene, ethyltoluene, ethylxylenes, hemimellitene, pseudocumene, 55 prehnitene, isodurene, diethylbenzenes, isoamylbenzene and the like. Suitable aromatic hydrocarbon fractions can be obtained by the selective extraction of aromatic naphthas from hydroforming operations as distillates or bottoms, from cyclo stock fractions of cracking operations, etc.

Also may be employed certain alkyl naphthalenes which are liquid under the polymerization reaction con-

ditions, for example, 1-methylnaphthalene, 2-isopropyl-naphthalene, 1-n-amylnaphthalene and the like, or commercially produced fractions containing these hydrocarbons.

The catalysts include azo or peroxide catalyst such as, for example, various organic peroxides, including aliphatic, aromatic, heterocyclic and acyl peroxides, such as diethyl peroxide, tertiary butyl hydroperoxide, dibenzoyl peroxide, dimethylthienyl peroxide, dicyclohexyl peroxide, dilauroyl peroxide and urea peroxide. These are mentioned by way of non-limiting examples of suitable organic peroxides. Other catalysts include sodium bisulfite, diethyl sulfoxide, ammonium persulfate, alkali metal perborate, azo compounds, such as alpha, alpha-azodiisobutyronitrile, etc.

recovered and the copolymer exhibited excellent detergent properties.

#### EXAMPLE V

In a benzene solution containing 0.2% alpha, alpha'-azodiisobutyronitrile 2 mols of stearyl methacrylate, 1 mol of bischloroethylvinyl phosphonate and 1 mol of omega-hydroxyamyl methacrylate were added and the mixture was heated for 24 hours at 80° C. At the end of the reaction time an oil-soluble copolymer of stearyl methacrylate/bis - chloroethylvinyl phosphonate/omega-hydroxyamyl methacrylate having a molecular weight of 150,000 was recovered and the copolymer exhibited excellent detergent properties.

Following the above procedure, the following copolymers were prepared:

| Example | Omega-hydroxy C <sub>8-7</sub> acrylate ester | C <sub>8-20</sub> alkyl acrylate ester | Optional monomer   | Solvent | Catalyst                    | Temp., °C. | Molecular weight of polymer |
|---------|-----------------------------------------------|----------------------------------------|--------------------|---------|-----------------------------|------------|-----------------------------|
| VI      | ω-Hydroxyamyl acrylate                        | Stearyl methacrylate                   |                    | Benzene | Ditertbutyl peroxide        | 90         | 250,000                     |
| VII     | ω-Hydroxyhexyl methacrylate                   | do                                     |                    | do      | α, α'-Azodiisobutyronitrile | 80         | 150,000                     |
| VIII    | do                                            | do                                     | Triallyl phosphate | Heptene | do                          | 80         | 100,000                     |
| IX      | ω-Hydroxyamyl methacrylate                    | do                                     | Vinyl pyrrolidone  | Benzene | do                          | 80         | 200,000                     |
| X       | do                                            | Lauryl methacrylate                    | Vinyl stearate     | do      | do                          | 90         | 250,000                     |

The following examples are illustrative of the present invention.

#### EXAMPLE I

In a benzene solution containing 0.2% alpha, alpha'-azodiisobutyronitrile 2 mols of stearyl methacrylate and 1 mol of omega-hydroxyamyl methacrylate were added and the mixture was heated for 24 hours at 80° C. At the end of the reaction time an oil-soluble copolymer of stearyl methacrylate/omega - hydroxyamylmethacrylate having a molecular weight of 155,000 was recovered and the copolymer exhibited excellent detergent properties.

#### EXAMPLE II

In a benzene solution containing 0.2% alpha, alpha'-azodiisobutyronitrile 1.1 mols of stearyl methacrylate, 1.9 mols of lauryl methacrylate and 1 mol of omega-hydroxyamyl methacrylate were added and the mixture was heated for 24 hours at 80° C. At the end of the reaction time an oil-soluble copolymer of stearyl methacrylate/omega-hydroxyamyl methacrylate having a molecular weight of 400,000 was recovered and the copolymer exhibited excellent detergent properties.

#### EXAMPLE III

In a benzene solution containing 0.2% alpha, alpha'-azodiisobutyronitrile 2 mols of stearyl methacrylate and 1 mol of 1,3-dimethyl-omega-hydroxyamyl methacrylate were added and the mixture was heated for 24 hours at 80° C. At the end of the reaction time an oil-soluble copolymer of stearyl methacrylate/1,3-dimethyl-omega-hydroxyamyl methacrylate having a molecular weight of 155,000 was recovered and the copolymer exhibited excellent detergent properties.

#### EXAMPLE IV

In a benzene solution containing 0.2% alpha, alpha'-azodiisobutyronitrile 2 mols of stearyl methacrylate, 1 mol 2-methyl-5-vinylpyridine and 1 mol of omega-hydroxyamyl methacrylate were added and the mixture was heated for 24 hours at 80° C. At the end of the reaction time an oil-soluble copolymer of stearyl methacrylate/2 - methyl-5-vinylpyridine/omega - hydroxyamyl methacrylate having a molecular weight of 100,000 was

When desired, additional improvements with respect to oxidation stability and scuffing inhibition can be imparted to the oil compositions containing the copolymers of this invention by incorporating small amounts (0.01% - 2%, preferably 0.1% - 1%) of phenolic antioxidants such as alkylphenols, e.g., 2,6-ditertbutyl-4-methylphenol or p,p'-methylene bisphenols such as 4,4'-methylene bis (2,6-ditertbutylphenol) or arylamines such as phenyl-alpha-naphthylamine and mixtures thereof. Anti-scuffing agents include organic phosphites, phosphates, phosphonates and their thio-derivatives, such as C<sub>3-18</sub> alkyl phosphites, or phosphonates, e.g., di- and tributyl, octyl, lauryl, stearyl, cyclohexyl, benzyl, cresyl, phenyl, phosphites or phosphates, as well as their thio-derivatives, P<sub>2</sub>S<sub>5</sub>-terpene reaction product, e.g., P<sub>2</sub>S<sub>5</sub>-pine oil reaction product and alkali metal salts thereof such as a potassium salt of a P<sub>2</sub>S<sub>5</sub>-terpene reaction product, phosphonates such as dibutyl methanephosphonate, dibutyl trichloromethane-phosphonate, dibutyl monochloromethanephosphonate, dibutyl chlorobenzene-phosphonate, and the like. The full esters of pentavalent phosphorous acids such as triphenyl, tricresyl, triauryl and tristearyl ortho-phosphates or potassium salt of P<sub>2</sub>S<sub>5</sub>-terpene reaction product are preferred.

The polymeric additives of this invention improve various mineral oil products by the incorporation of a minor amount (0.01% to 5%, preferably 0.1% to 3% by weight) of the additive. Thus, they may be used to improve transformer oils, turbine oils, mineral lubricating oils, industrial oils and the like. Suitably such lubricating oils range from SAE 5W viscosity grade to SAE 140 grade and are derived from paraffinic, naphthenic or asphaltic base crudes. Representative oils are refined high viscosity index mineral oils having a viscosity of 100° F of 100 to 250 SUS. A typical mineral lubricating oil (X) of this type had the following properties:

|                                  |     |
|----------------------------------|-----|
| Gr. ° API, 60/60° F.             | 32  |
| Flash, ° F.                      | 370 |
| Viscosity Index (Dean and Davis) | 93  |
| Viscosity, SUS at 100° F.        | 103 |

The following non-ash compositions are representative of this aspect of the invention.

|                                                     |             |
|-----------------------------------------------------|-------------|
| Composition A:                                      | Percent wt. |
| Example I copolymer                                 | 2           |
| Mineral lubricating oil (X)                         | Balance     |
| Composition B:                                      |             |
| Example II copolymer                                | 2           |
| Mineral lubricating oil (X)                         | Balance     |
| Composition C:                                      |             |
| Example III copolymer                               | 2           |
| Mineral lubricating oil (X)                         | Balance     |
| Composition D:                                      |             |
| Example IV copolymer                                | 2           |
| Mineral lubricating oil (X)                         | Balance     |
| Composition E:                                      |             |
| Example V copolymer                                 | 2           |
| Mineral lubricating oil (X)                         | Balance     |
| Composition F:                                      |             |
| Example I copolymer                                 | 3           |
| 4,4'-methylene bis(2,6-di- <i>tert</i> butylphenol) | 1           |
| Mineral lubricating oil (aviation oil 1100 grade)   | Balance     |
| Composition G:                                      |             |
| Example I copolymer                                 | 5           |
| 4,4'-methylene bis(2,6-di- <i>tert</i> butylphenol) | 0.5         |
| Tricresyl phosphate                                 | 0.8         |
| Mineral lubricating oil (X)                         | Balance     |

In order to demonstrate the utility and improved properties of this invention, the compositions identified in Table I were tested in the Chevrolet V-8 Sludging Test, modified EX-3 test described in CRC Progress Report No. 3, June 1, 1957, and the results were as follows:

Table I

| Composition                                                                                                                 | Active group                                                                        | Piston <sup>a</sup> varnish | Total <sup>b</sup> varnish | Total <sup>c</sup> sludge | Final <sup>d</sup> rating | Percent oil ring plugging | Percent vise. increase at 100° F. |
|-----------------------------------------------------------------------------------------------------------------------------|-------------------------------------------------------------------------------------|-----------------------------|----------------------------|---------------------------|---------------------------|---------------------------|-----------------------------------|
| 1. Composition A (present invention)                                                                                        | $-\text{O}-\text{C}_5-\text{OH}$                                                    | 9.3                         | 45.1                       | 79.1                      | 94.8                      | 5                         | 13                                |
| Composition B (present invention)                                                                                           | $-\text{O}-\text{C}_5-\text{OH}$                                                    | 8.3                         | 40.8                       | 72.7                      | 86.2                      | 5                         | 13                                |
| 2. Mineral oil (X) plus 2% copolymer stearyl methacrylate and monomethacrylate ester of hexylene glycol (M.W. 143,000).     | $-\text{O}-\text{C}(\text{C})(\text{C})-\text{COH}$                                 | 8.3                         | 40.0                       | 60                        | 77.6                      | 13                        | 50                                |
| 3. Mineral oil (X) plus 2% copolymer stearyl methacrylate and hydroxyethyl methacrylate (M.W. 230,000).                     | $-\text{O}-\text{C}_2-\text{OH}$                                                    | 8.8                         | 41.6                       | 63.6                      | 81.5                      | 16                        | 23                                |
| 4. Mineral oil (X) plus 2% copolymer of vinyl pyrrolidone and lauryl methacrylate (M.W. 500,000).                           | $-\text{CH}_2-\text{CH}_2-\text{CH}(\text{CH}_2-\text{C}=\text{O})-\text{N}$        | 8.5                         | 40.1                       | 70.2                      | 84.0                      | 25                        | 27                                |
| 5. Mineral oil (X) plus 2% copolymer of lauryl methacrylate, stearyl methacrylate, 2-methyl-5-vinylpyridine (M.W. 500,000). |  | 8.5                         | 39.5                       | 61.0                      | 77.6                      | 79                        | 23                                |

<sup>a</sup> 10, perfect. <sup>b</sup> 50, perfect. <sup>c</sup> 100, perfect.

<sup>d</sup> 100, perfect.

#### References Cited by the Examiner

#### UNITED STATES PATENTS

|           |       |                |          |
|-----------|-------|----------------|----------|
| 2,892,790 | 6/59  | Stuart et al.  | 252—56   |
| 2,892,792 | 6/59  | Stewart et al. | 252—56   |
| 2,892,819 | 6/59  | Stewart et al. | 252—56 X |
| 2,913,439 | 11/59 | Bondi et al.   | 252—56 X |
| 2,927,013 | 3/60  | Lowe           | 44—62    |
| 2,949,445 | 8/60  | Blake          | 260—86.1 |
| 2,980,658 | 4/61  | Ham            | 260—86.1 |
| 2,994,663 | 8/61  | Lowe et al.    | 252—56   |

#### FOREIGN PATENTS

590,443 1/60 Canada.

DANIEL E. WYMAN, Primary Examiner.

JULIUS GREENWALD, JOSEPH R. LIBERMAN,  
Examiners.

Lubricating compositions of this invention are particularly applicable for high temperature, high speed use as in aviation engines, automotive engines, truck engines as well as industrial equipment.

We claim as our invention:

1. A mineral lubricating oil composition consisting essentially of a major amount of mineral lubricating oil and from about 0.01% to 5% by weight of an oil-soluble copolymer of a  $\text{C}_{12-20}$  alkyl methacrylate and an ester of methacrylic acid and an alpha, omega  $\text{C}_{5-7}$  alkanediol in the ratio of 1:10 to 10:1, respectively, said copolymer having a molecular weight of from 10,000 to 500,000.

2. A mineral lubricating oil composition consisting essentially of major amount of mineral lubricating oil and from about 0.01% to 5% by weight of an oil-soluble copolymer of a  $\text{C}_{12-20}$  alkyl methacrylate and an ester of methacrylic acid and 1,5-pentanediol in the ratio of 1:10 to 10:1, respectively, said copolymer having a molecular weight of from 10,000 to 500,000.

3. A mineral lubricating oil composition consisting essentially of a major amount of mineral lubricating oil and from about 0.01% to 5% by weight of an oil-soluble copolymer of stearyl methacrylate and an ester of methacrylic acid and 1,5-pentanediol in the ratio of 1:10 to 10:1, respectively, said copolymer having a molecular weight of from 10,000 to 500,000.

4. A mineral lubricating oil composition consisting essentially of a major amount of mineral lubricating oil and from about 0.01% to 5% by weight of an oil-soluble copolymer of stearyl methacrylate, lauryl methacrylate, an ester of methacrylic acid and 1,5-pentanediol in the ratio of 1:10 to 10:1, respectively, said copolymer having a molecular weight of from 10,000 to 500,000.